

## 1

3,276,890

## ASPHALT PAVING COMPOSITION

Jack M. Reese, West Point, Miss., assignor to Renrock, Inc., West Point, Miss., a corporation of Mississippi  
No Drawing. Filed Apr. 15, 1963, Ser. No. 272,878  
6 Claims. (Cl. 106—283)

This invention relates to asphalt concrete, particularly for paving.

Reference should be made to the Asphalt Handbook (1960 edition) published by the Asphalt Institute of College Park, Maryland, from which the terminology used herein is taken, with minor exceptions.

Broadly, asphalt concretes are made up of an aggregate of a size range and distribution suited to the service intended, bound by an asphaltic cement or binder. The particular aggregate used in this invention is not a matter of significance since this invention is generally applicable to all aggregates. If an aggregate can be used in an asphaltic concrete of another kind, it can be used with my invention. The selection of aggregates is an operation more involved than is apparent to the average observer and is the subject of much technical literature. Extensive information on the selection of aggregates may be found in the Handbook on Bituminous Construction published by the Barber-Greene Company and the Asphalt Handbook indicated above.

In determining the amount of asphalt required for binding the aggregate, it should be remembered that the asphalt should adequately bind and stabilize the aggregate. Additionally, it must seal the pavement against the destructive action of air and water. On the other hand, an excessive amount of asphalt will impair the stability of the concrete body and lead to a slick surface. The amount of asphalt in the surface course is particularly critical. When the surface course is porous for any reason, including the use of insufficient binder, air will penetrate into the structure and oxidize the binder. Oxidation results in hardening of the asphalt, and when its viscosity reaches a value somewhat above  $1 \times 10^7$  poises at 77° F. the asphalt will no longer serve as a satisfactory binder at low atmospheric temperatures. When the binder becomes too hard, the pavement surface erodes under the action of traffic. An inadequacy of 0.5% asphalt in a mixture may result in a road that requires excessive maintenance. From this, it will be recognized that it is desirable to employ asphalts of lesser viscosity and superior oxidation resistance for best results.

The foregoing criteria for the selection of asphalts are well known in the art. It is also known that the lower viscosity asphalts do not adequately bind the aggregate by reason of their fluent nature. Accordingly, it is customary to increase the viscosity of the asphalt by adding thereto a quantity of finely divided mineral matter, known as a filler or stabilizing agent. It has been observed that the same result is obtained by using a harder asphalt so far as the immediate result is concerned but such harder asphalts may be expected to have a shorter life. The mineral filler is frequently obtained by screening the aggregate to be employed to obtain a fraction passing the 200 mesh screen. Among the minerals that have been recognized as acceptable as fillers are: limestone, silica, Portland cement, clay, slate, talc, mica, diatomaceous earth and asbestos. It has also been recognized that there

## 2

is a great variation in the effectiveness of fillers; the minerals named are in an ascending order of effectiveness with asbestos recognized as having more than four times the value of limestone on a volume basis.

Not only is it important to test mineral aggregate and asphalt separately, but tests should also be made on the combinations of these materials to establish the proper proportions and characteristics for asphalt concrete mixtures. The Asphalt Handbook at pages 36 through 45 and 67 lists five recognized testing methods. Although no two methods can be related with mathematical precision, the results are generally comparable. The product of this invention has been tested by the Marshall method; this procedure is the official one used by the United States Corps of Engineers for designing air field paving.

Due to the necessity for procuring the aggregate at a point relatively close to the point of consumption, because of the great weight and bulk of material handled, a substantial degree of latitude must be employed in the selection of the optimum blends of ingredients for use at any specific location. The choice of suitable mixtures satisfying acceptable requirements is referred to as the design of a paving mixture.

This invention is based upon the discovery that asphalt concretes of unusually high stability value (as determined by the Marshall method) are produced by the use of a mineral filler consisting of Selma chalk limestone. Selma chalk limestone is the name of a geological stratum found over a wide area of the southern United States and particularly in the vicinity of Selma, Alabama, from which it takes its name. As is also indicated by the other portion of its name, it is primarily calcium carbonate of a soft, chalky nature. A typical analysis is:

|                        | Percent |
|------------------------|---------|
| 35 Silica              | 7.75    |
| Iron oxide             | 2.05    |
| Aluminum oxide         | 7.25    |
| Phosphorous            | 0.21    |
| Sulphates              | 0.82    |
| 40 Magnesium carbonate | 1.52    |
| Calcium carbonate      | 80.40   |

A similar stratum, probably of the same geologic origin extends from southwestern Arkansas westward to the vicinity of Sherman, Texas, and thence in a generally southerly direction through eastern Texas.

The material is widely sold in finely ground condition under the name of agricultural limestone. It is usually ground to pass substantially through a No. 4 sieve and more than half will pass through a No. 40 sieve. Since asphalt concretes are normally intended to bear comparatively heavy loads, it is axiomatic that mineral aggregates should have very substantial crushing strength, far in excess of that possessed by Selma chalk limestone. Also, since conventional limestone has the lowest satisfactory value as a mineral filler, it is surprising to find this particular limestone so useful in this respect.

As stated, the agricultural limestone of commerce made from Selma chalk limestone is supplied ground to substantially all pass through a No. 4 screen. About 20% usually passes a No. 200 screen and it is this portion which is immediately available as mineral filler, the remaining 80% acting as fine aggregate. However, substantial internal grinding takes place during the batching and mix-

ing operations employed during the production of asphalt concrete as it is usually made, due to the softness of the Selma limestone in relation to the hard aggregates needed for load bearing applications of the concrete. Consequently, it is assumed that a larger amount of the agricultural limestone is found ultimately in the filler than might be assumed from the initial sieve analysis of the agricultural limestone.

In a typical application, where a range of 3 to 8% mineral filler would be used, it has been found that 10% agricultural limestone is sufficient. Although the 10% used exceeds the 8% normal range, only 20% of this or 2% is available in the filler range, yet the results are superior to those obtained when dust from a hard aggregate is used as the filler.

Although asphalt may be admixed with aggregate and mineral filler in a number of ways as by hot mixing, as cut-back, that is, diluted with a solvent, or as an emulsion. Further, the emulsion may make use of either an anionic or cationic emulsifying agent or the emulsion may be inverted, with the water as the internal phase. In the practice of this invention, very gratifying results have been obtained in the use of an anionic emulsion, particularly of the slow setting type. Heretofore, asphalt concretes made by the hot mix method have been considered so superior for general paving that many State highway departments specify their use to the exclusion of other types. Following the teachings of this invention and using an anionic asphalt emulsion, asphalt concretes meeting the highest duty requirements can be produced without difficulty. Since the mixing apparatus needed for use with an emulsified asphalt is much less complex and less expensive, it is evident that great savings can be made.

In the tables that follow, there is demonstrated the manner in which suitable levelling course and surface course paving materials are designed.

The first step is designing the asphalt concrete is to obtain a sieve analysis of the solid material to be employed. Table I shows this. Table II shows the specification to which the asphalt emulsion is produced; this is the type identified as SS-1.

TABLE I.—SIEVE ANALYSIS OF MATERIAL

| Sieves  | Material |      |                       |
|---------|----------|------|-----------------------|
|         | Gravel   | Sand | Agriculture Limestone |
| 3/4"    | 100      |      |                       |
| 1/2"    | 86.3     |      |                       |
| 5/8"    | 63.3     |      |                       |
| No. 4   | 13.4     | 100  | 100                   |
| No. 10  | 1.3      | 95.2 | 97.0                  |
| No. 40  |          | 77.2 | 86.0                  |
| No. 80  |          | 38.6 | 60.0                  |
| No. 200 |          | 2.6  | 41.0                  |
|         |          | 0.2  | 19.0                  |

The amounts listed under the respective material columns are the percentage amount passing each sieve.

TABLE II.—SPECIFICATIONS ON EMULSION ASTM

|                            |                                                  |
|----------------------------|--------------------------------------------------|
| Furol viscosity in seconds | 77° F., 40-400.                                  |
| Asphalt content            | Min. 60%.                                        |
| Settlement test            | 5%—5 days max.                                   |
| Demulsibility              | Normal 10% solution of calcium chloride, 2% max. |
| Sieve test                 | Max. .05% retained.                              |
| Miscibility                | Must mix with water.                             |
| Cement mix test            | Min. 2% (ability to mix with fines).             |
| Asphalt (to be emulsified) | Penetration, 77° F., 100-200.                    |

|                                     |                     |
|-------------------------------------|---------------------|
| Percent soluble in carbon disulfide | 97.0% min.          |
| Percent ash                         | Max. 2%.            |
| Ductility, 77° F.                   | 40 centimeters min. |
| Specific gravity, 77° F.            | 1 min.              |

Next, tentative proportions of the solid ingredients are selected and made up and a new sieve analysis made of the mixed ingredients as shown in Tables III-A and III-B.

TABLE III-A.—PROPORTIONS OF MATERIALS AND COMPOSITE GRADATION

|    | Design   | Leveling Course | Surface |
|----|----------|-----------------|---------|
| 15 | Gravel   | 50.0            |         |
|    | Sand     | 40.0            | 75.0    |
|    | Ag. Lime | 10.0            | 25.0    |

TABLE III-B

|    | Sieves  | Leveling Course | Surface |
|----|---------|-----------------|---------|
| 20 | 3/4"    | 100             |         |
|    | 1/2"    | 93.2            |         |
|    | 5/8"    | 81.7            |         |
|    | No. 4   | 54.5            | 100     |
|    | No. 10  | 40.2            | 95.7    |
| 25 | No. 40  | 21.4            | 79.4    |
|    | No. 80  | 5.1             | 44.0    |
|    | No. 200 | 2.0             | 12.3    |
|    |         |                 | 5.0     |

The amounts listed under the respective material columns are the percentage amount passing each sieve.

Multiple samples are made with several asphalt-to-solids ratios in what are deemed to be in the acceptable range. These are tested according to ASTM Standard D1559.

TABLE IV-A.—PROPORTIONS OF MATERIALS AND PHYSICAL PROPERTIES OF MIXES, LEVELING COURSE

| Mix No. | A                       | B     | C     | Sp. Gr. of Material |
|---------|-------------------------|-------|-------|---------------------|
| 40      | 46.0                    | 45.0  | 45.0  | 2.550               |
|         | 36.8                    | 36.4  | 36.0  | 2.618               |
|         | 9.2                     | 9.1   | 9.0   | 2.778               |
|         | 8.0                     | 9.0   | 10.0  | 1.010               |
|         | 2,308                   | 2,276 | 2,245 |                     |
|         | 2,227                   | 2,219 | 2,234 |                     |
|         | 96.5                    | 97.5  | 99.5  |                     |
|         | 948                     | 898   | 702   |                     |
|         | 7                       | 9     | 19    |                     |
| 45      | Percent Moisture To Mix | 4.2   | 5.2   | 4.7                 |

TABLE IV-B.—PROPORTIONS OF MATERIALS AND PHYSICAL PROPERTIES OF MIXES, SURFACE COURSE

| Mix No. | A                       | B     | C     | Sp. Gr. of Material |
|---------|-------------------------|-------|-------|---------------------|
| 50      | 68.2                    | 67.5  | 66.8  | 2.618               |
|         | 22.8                    | 22.5  | 22.2  | 2.778               |
|         | 9.0                     | 10.0  | 11.0  | 1.010               |
|         | 2,316                   | 2,284 | 2,252 |                     |
|         | 2,110                   | 2,129 | 2,201 |                     |
|         | 91.1                    | 93.2  | 97.7  |                     |
|         | 1,973                   | 2,109 | 2,708 |                     |
|         | 6                       | 10    | 12    |                     |
|         | Percent Moisture To Mix | 8.0   | 8.4   | 8.2                 |

The foregoing tests and calculations were carried out under the supervision of Bruce G. Marshall, originator of the standard test. On the basis of the experimental results, he suggested that 8.5% of emulsion be used in the leveling course, to produce a Stability Rating of about 925 and a Flow Value of 8. For the surface course, the recommended amount of emulsion was 9.0. However, because the Stability Rating was greater than required, it was recommended that the limestone be decreased from 25% to 15% with corresponding increase in the amount of sand. As will be noted from Table IV-9 of the Asphalt Handbook, for heavy traffic, a minimum Stability Value of 750 is desired along with a Flow Value of 8. Since the asphalt concrete of this particular design was intended

for paving city streets, the minimum acceptable flow value was sought. For lighter traffic a Stability Value of 500 is recognized as acceptable but with the trend toward increasingly heavy traffic, the higher Stability Values are favored. As shown by the results of Tables IV-A and B, the Stability Values obtained by the use of Selma chalk limestone ground to pass a No. 4 sieve tend to exceed the expectations of an especially skilled designer of asphaltic compositions.

Utilizing recognized standards for the selection of the kind, amount and size distribution of aggregate, recognized standards for the kind and amount of asphalt and established performance standards for asphalt concretes this invention resides in the use of Selma chalk limestone as the mineral filler for the asphalt. Desirably, it contemplates the inclusion of 10 to 15% of such limestone in the fine aggregate as well. Also, although it has been recognized that the hot-mix process of formulating asphalt concretes is most desirable, the use of this limestone yields excellent results with anionic emulsions thereby reducing the cost of producing acceptable paving mix.

I claim:

1. In an asphalt concrete containing an aggregate and asphalt, the improvement consisting of Selma chalk limestone as the asphalt filler.
2. An asphalt concrete containing as essential ingredients: an aggregate of size distribution suitable to the use intended for said concretes, the asphaltic residue of an anionic asphalt emulsion and finely ground Selma chalk limestone in an amount sufficient to form the filler of the concrete.

10

15

20

25

30

35

3. An asphalt concrete containing as essential ingredients: an aggregate of size distribution suitable to the use intended for said concretes, asphalt and finely ground Selma chalk limestone in an amount sufficient to form the filler of the concrete.

4. An asphalt concrete containing as essential ingredients: an aggregate of size distribution suitable to the use intended for said concretes, asphalt and finely ground Selma chalk limestone, a portion of said being of fine aggregate dimension and a further portion being finer than No. 200 mesh to act as filler for said asphalt.

5. An asphalt concrete having a Stability Value in excess of 500 as determined by the Marshall method wherein substantially all of the mineral filler under No. 200 mesh and a minor but significant amount of the fine aggregate is made up of Selma chalk limestone.

6. A composition as in claim 5 wherein the asphalt is the asphaltic residue of an anionic emulsion.

#### References Cited by the Examiner

#### UNITED STATES PATENTS

|           |         |                  |            |
|-----------|---------|------------------|------------|
| 2,086,581 | 7/1937  | Smith            | 106—281 XR |
| 2,773,777 | 12/1956 | Alexander et al. | 252—311.5  |
| 3,046,149 | 7/1962  | Moore et al.     | 106—273    |
| 3,052,639 | 9/1962  | Wright et al.    | 106—96     |

ALEXANDER H. BRODMERKEL, Primary Examiner.

MORRIS LIEBMAN, Examiner.

J. B. EVANS, Assistant Examiner.